

June 12, 1923.

1,458,631

P. E. SABINE

SOUND ABSORBING PLASTER

Filed April 29, 1921

*Fig. 1.*



*Fig. 2a.*



*Fig. 2.*



*Fig. 3.*



Witness:

John Enders

Inventor:

Paul E. Sabine,

by Wallace R. Lane

Atty.

## UNITED STATES PATENT OFFICE.

PAUL E. SABINE, OF GENEVA, ILLINOIS, ASSIGNOR OF ONE-HALF TO RIVERBANK LABORATORIES, OF GENEVA, ILLINOIS.

## SOUND-ABSORBING PLASTER.

Application filed April 29, 1921. Serial No. 465,372.

To all whom it may concern:

Be it known that I, PAUL E. SABINE, a citizen of the United States, residing at Geneva, in the county of Kane and State 5 of Illinois, have invented certain new and useful Improvements in Sound-Absorbing Plaster, of which the following is a specification.

This invention relates to the preparation 10 and application of a special plaster of such nature that it may be applied to walls, ceilings, or the like, with ordinary plastering tools, and when set or hardened will have the property of absorbing sound to a much 15 greater degree than plasters heretofore known.

As is well known it is oftentimes a question of considerable importance and necessity to so construct buildings, rooms, and 20 the like, as to reduce to the minimum the penetration thereinto of audible sound waves. The necessity for this more often occurs in such buildings as auditoriums, concert halls, theaters, and the like, where 25 it is of prime importance to secure proper acoustical conditions and to reduce the noise therein from external sources.

It has been long known that porous surfaces have the property of absorbing a 30 large percentage of the sound that may be incident upon them, and various methods of securing structural materials possessing porosity have been devised. In actual practice, however, none of these materials can 35 be applied as plaster to the walls, ceilings, and the like, since it has heretofore been impossible to produce a mortar of such consistency and nature that it can be handled with plastering tools, and which will set 40 into a porous body. Porosity has heretofore been secured by using as an aggregate or body material a granular substance, from which the finest particles have been screened or removed, and such a small percentage of 45 bonding material used that cementing occurs only at the points of contact, so as to leave inter-communicating pores throughout the body of the hardened material. Actual experiment, however, shows that a 50 mixture of this character cannot be applied as a plastic material, since the requisite porosity calls for a mixture too dry to be handled as ordinary mortar or plaster.

Among the objects of my invention are

to provide a plaster of such nature that it 55 may be applied to walls, ceilings, and the like, with ordinary plastering tools, and which when hardened will absorb sound to a greater degree than possible with the plasters heretofore known; further the 60 proper choice of materials and the method of mixing and applying the same in such manner as to produce a plaster or mortar which is capable of being applied in the usual manner, and when set will be sufficiently porous to be highly absorbent of sound; further to select an aggregate or body material, the shape of the separate particles of which are such as to prevent 65 close packing; further to produce a bonding 70 material of such nature that the voids between the body particles are not completely filled in the process of trowelling and finishing but the bonding material therein is of a porous and cellular structure; further the 75 provision of a bonding material which will form elastic surface films so that in mixing with the aggregate a large number of minute air particles are formed, which break in the setting of the plaster, giving a 80 cellular and porous nature to the hardened product; further to produce a plaster in which the aggregate consists of particles having a large number of more or less sharp 85 projections to promote porosity between the various particles; further to provide a novel bonding material for the aggregate; further to make possible a more simple, highly efficacious and cheaper produced plaster for absorbing sound; and such further objects, 90 advantages and capabilities as will later more fully appear.

While I have shown in the accompanying drawings, certain forms of aggregate, I wish it to be understood that the same is 95 illustrative only, and not to be considered as limiting the scope of my invention, since other forms of aggregate may be used.

In the drawings:

Fig. 1 shows in separated relation various 100 particles of aggregate having a large number of sharp projections.

Fig. 2 is a cross section showing how the irregularly shaped particles of aggregate prevent close packing and form air spaces 105 therebetween prior to having the bonding material added thereto.

Fig. 2a is a view similar to Fig. 2, but

showing in magnified form the bonding material applied in the spaces between the irregular particles of aggregate and the cellular and porous nature of the bonding material.

Fig. 3 is a diagram illustrating by means of curves the results of careful scientific tests made to determine the efficiency of my improved plaster as a sound absorber.

For a bonding material, I use a well known material known as Sorel cement, consisting of a mixture of a solution of magnesium chloride and magnesium oxide. When mixed to form a paste, these materials will harden into an extremely hard and tenacious solid. There are other known methods of producing the compound thus formed, by the use of other salts of magnesium, of which I may avail without departing from the spirit of my invention. To the solution of magnesium chloride is added a very small amount of glue, gelatine, or other material, which with water will form a colloidal solution. One per cent by weight of glue is sufficient for the purpose. The addition of even this small amount of colloidal material is of importance in securing the desired result. The presence of the glue or other colloidal material causes a marked foaming action in the mixing of the mortar. This action produces a wet mixture of the proper consistency to be handled with plastering tools, and yields a hardened product sufficiently porous to be highly absorbent of sound.

As an aggregate, I preferably use the granulated slag from iron blast furnaces. This material is prepared by passing the molten slag from the furnace directly into cold water. The expansive force of the steam thus formed, breaks the slag into small particles, and the cellular structure of the slag is such that these particles have each numerous sharp projecting points. Figure 1 represents the character of these particles, which are designated at 1. The advantage of this material lies in the fact that the shapes of the particles render close packing impossible, and allows liberal intervening spaces which are filled with the porous bonding material produced as heretofore described, the whole constituting a hard porous material which is highly absorbent of sound.

While I have mentioned granulated slag, I wish any other material of such shape and nature as to accomplish the results desired, to be understood as falling within the scope of my invention.

As an instance of the employment of the foregoing materials, the following example of their use in the preparation of a sound absorbing plaster is given.

To a solution in water of magnesium chloride of density 20° Baumé, is added 1% by weight of glue. Equal volumes of

the resulting mixture and dry magnesium oxide are mixed to form a thin paste. Into this paste, four volumes of the granulated slag is thoroughly worked.

One of the important features of my invention consists in the peculiar combination of properties possessed by the binding material and the aggregate. Experiment shows that the use in the same proportions of other ingredients such as are ordinarily used in plasters would give a mixture entirely too poor in bonding material to adhere to a wall or ceiling. In mixing this product, the sharp particles of the slag, acting upon the slightly gelatinous paste produces a large number of minute air bubbles throughout the mixture. The effect is similar to that produced by beating the white of an egg. The presence of these bubbles accomplishes a two fold purpose. It imparts to the wet mixture the proper consistency for handling, and to the hardened product both a porous and cellular structure which renders it highly sound absorber. The character of the slag particles is also important, since without the projecting points, the particles would tend to pack more closely, thus counteracting the effect just described.

When a train of sound waves is incident upon a reflecting surface, a certain definite fraction of this incident energy is reflected, another definite fraction absorbed, and the remainder is transmitted. For fairly rigid massive walls the fraction transmitted is small in comparison with that reflected and absorbed so that for practical purposes the sum of the reflected and absorbed sound energies is equal to the incident energy. The merits of any surface as a sound absorber may be expressed by the fraction of the incident sound energy that is absorbed. The per cent of sound energy absorbed is independent of the intensity of the sound and depends only upon the pitch of the sound and the nature of the surface. (See Rayleigh—Theory of Sound, Vol. II, page 332 and following (1896)).

Careful scientific tests have been made to determine the efficiency of this material as a sound absorber. The results of these tests are shown in Figure 3. The abscissæ are the notes ranging from the second octave below middle C to the fourth octave above middle C. The ordinates are the per cents of sound absorbed. Curve 1 represents the absorption of a surface of two coats of this product made as described above and applied by a journeyman plasterer to a wall composed of gypsum block. Curve 2 represents the percentage of sound energy absorbed by two coats of the same material applied to a scratch coat of brown plaster upon metal lath. Curve 3 represents the absorption of sound by a wall finished with a hard surface of ordinary gypsum plaster.

Having now described my invention, I claim:—

1. A sound absorbent plaster for walls, ceilings, and the like, comprising granular particles of irregular shape to prevent close packing and leave voids therebetween, and a bonding material of such nature as to not completely fill the voids between said particles, said plaster being capable of application directly to a wall, ceiling, or the like with ordinary plastering tools.
2. A sound absorbent plaster for walls, ceilings, and the like, comprising granular particles having a large number of sharp projecting points, and a bonding material of such nature as to not completely fill the voids between said particles, said plaster being capable of application directly to a wall, ceiling, or the like with ordinary plastering tools.
3. A sound absorbent plaster for walls, ceilings, and the like, comprising granular particles of irregular shape to prevent close packing and leave voids therebetween, and a bonding material of such nature as to not completely fill the voids between said particles, said plaster being capable of application directly to a wall, ceiling, or the like with ordinary plastering tools, and when hardened will absorb more than twelve per cent of sound lying in the range of pitch between middle C and the fourth octave above middle C, when applied in thicknesses of one half inch or more.
4. A sound absorbent plaster comprising granular particles of irregular shape, and a bonding material which when being mixed with said granular particles forms a large number of minute bubbles throughout the mixture, to permit the same to be applied as a plaster to walls, ceilings and the like and set into a hard porous product possessing the property of absorbing more than twelve per cent of sound lying in the range of pitch between middle C and the fourth octave above middle C, when applied in thicknesses of one half inch or more.
5. A sound absorbent plaster comprising granular particles having sharp projecting

points which prevent close packing, and a bonding material which when being mixed with said granular particles forms a large number of minute bubbles throughout the mixture, to permit the same to be applied as a plaster to walls, ceilings and the like and set into a hard porous product possessing the property of absorbing more than twelve per cent of sound lying in the range of pitch between middle C and the fourth octave above middle C, when applied in thicknesses of one half inch or more.

6. A sound absorbing plaster comprising body particles of granulated slag, a bonding material consisting of the product of reaction between magnesium oxide and a solution of magnesium chloride to which is added a small per cent of a substance of colloidal nature, so that said plaster may be applied in a plastic condition to walls, ceilings and the like, and when hardened will be porous and capable of absorbing more than twelve per cent of sound lying in the range of pitch from middle C to the fourth octave above middle C.

7. A plaster of the character described comprising granulated slag, and a bonding material consisting of the product of reaction between magnesium oxide and a solution of magnesium chloride to which is added a small percentage of a substance of colloidal nature, whereby the structure of the plaster is porous and sound absorbing.

8. A plaster of the character described comprising granulated slag, and a bonding material consisting of the product of reaction between magnesium oxide and a solution of magnesium chloride to which is added a small percentage of a gelatinous material, whereby the structure of the plaster is porous and sound absorbing.

In witness whereof, I hereunto subscribe my name to this specification in the presence of two witnesses.

PAUL E. SABINE.

Witnesses:

FREDERICK F. MASON,  
EDITH OLSON.